

# UNITED STATES PATENT OFFICE.

IRA E. FARR, OF WATERTOWN, NEW YORK.

## COMPOSITION PLUG.

1,259,502.

Specification of Letters Patent. Patented Mar. 19, 1918.

No Drawing.

Application filed March 12, 1917. Serial No. 154,289.

To all whom it may concern:

Be it known that I, IRA E. FARR, a citizen of the United States, residing at Watertown, in the county of Jefferson and State of New York, have invented certain new and useful Improvements in Composition Plugs, of which the following is a specification.

The invention relates to an improved plug or bushing capable of a wide field of use, although specifically adapted for supporting rolls of wrapping and other paper, and to the composition of which said plug is composed.

The composition of materials out of which the plug is composed preferably consists of a pulpy substance incorporated and thoroughly mixed with a hardening material, to which is added and intermixed a binding ingredient, all being thoroughly mixed and then pressed in any preferred manner in bushings of the desired shape.

The material or ingredients comprising the composition of which my improved plugs are made, consists of a pulp, preferably derived from old newspapers, waste paper and the like, commonly called "paper stock," a quantity of cement to harden the mass to a certain extent, a quantity of lime to coact with the cement as a binder, and water in sufficient quantity to render the composition pasty to a degree suitable for properly molding and compressing into a compact and smooth body.

Heretofore, plugs for paper rolls have usually been turned up out of wood, and bored out to receive shafts or rods upon which the rolls are mounted and rotatable as the paper is used. These wooden plugs are turned up in several standard sizes intended to snugly fit in the ends of the different size rolls of paper. As a rule, the wood from which the plugs are made is green or wet and the plugs invariably shrink when they become dried out, and many of the wooden plugs when thoroughly dried, crack or split, and are therefore unfit for use. Furthermore, a large proportion of the wooden plugs warp or otherwise get out of shape so that they do not properly fit the openings in the ends of the rolls, and the rolls are therefore liable to get out of shape or collapse, which interferes with the ready unwinding of the paper when wanted for wrapping purposes. My composition plugs are intended to replace the old wooden plugs

in common use, without increasing the cost of the plugs and at the same time my plugs, because of the nature of the ingredients comprising the composition, are not liable to shrink or get out of shape no matter how long they are used. My process or method will now be described.

In the process of preparing the composition, newspapers or other suitable waste paper are first beaten by the well-known pulp beaters until finely broken up. This pulp contains a liberal quantity of water in order to facilitate the beating. The next step consists of adding to the pulp approximately 40% in weight of a suitable cementitious substance, such as Portland cement or analogous substance, which is then mixed with the pulp by any suitable agitating means. The third step consists of adding approximately 10% in weight of finely powdered slaked lime and again agitating all of said ingredients until they are thoroughly incorporated and the whole becomes a relatively thick paste. The paper stock is in such proportion (about 60%) as to render the plugs fibrous and light, while the cement and lime act as binders, and at the same time tend to solidify the pulpy mass, and when the composition is suitably compressed, and allowed to dry and harden, the plugs will stand considerable crushing strain and rough handling without getting out of shape. By the use of the cement and lime the bodies of the plugs are more solid and are less liable to shrink or warp or otherwise get out of shape. After the composition is prepared as described, it is delivered to a machine (which is not illustrated as it forms no part of the present invention, it being understood that any of the conventional machines may be employed for this purpose), which is arranged to force and compress measured quantities of the composition into a mold, and during the molding operation practically all of the surplus water contained in the composition is squeezed out, so that when the plugs are ejected from the mold they are of predetermined uniform size and shape and they are also relatively hard and smooth, as well as comparatively tenacious and light. Following the molding of the plugs, the latter are artificially dried for an hour or two, and then they are ready for shipment and use.

The material of which the plugs are made

- is composed of wood pulp, preferably old paper stock, lime, cement, and water, as described, which is suitably mixed and worked until it becomes a relatively thick paste. 5 The relatively thick paste, composed of the ingredients above referred to, or their equivalents which will form a bushing of this general character are delivered to any of the well known types of forming machines, 10 which will automatically turn out the bushings in rapid order by pressing and forming the pasty substance into the desired formations.
- Having thus described the invention, what 15 I claim is:
1. The herein described plastic composition for molding plugs for paper rolls, consisting of a fluid wood pulp, powdered slaked lime, and cement, substantially as described. 20
  2. The herein described plastic composition for making plugs, consisting of old paper stock, slaked lime, cement, and water, substantially as described. 25
  3. The herein described plastic composition, consisting of old paper stock, sixty parts, finely powdered slaked lime, ten parts, and cement, thirty parts, and water substantially as described.
  4. A bushing of the character described 30 composed of a plastic composition consisting of paper stock, slaked lime and cement, and a fluid, substantially as described.

In testimony whereof I affix my signature.

IRA E. FARR.

**Copies of this patent may be obtained for five cents each, by addressing the "Commissioner of Patents, Washington, D. C."**